

## 1

3,833,649

 PROCESS FOR PRODUCING UNSATURATED  
CARBOXYLIC ACIDS

Masahiro Wada, Nishinomiya, Isao Yanagisawa, Ikeda,  
Michikazu Ninomiya, Kobe, and Takashi Ohara,  
Nishinomiya, Japan, assignors to Nippon Shokubai  
Kagaku Kogyo Co., Ltd., Osaka, Japan  
No Drawing. Filed Oct. 19, 1971, Ser. No. 190,661  
Int. Cl. C07c 51/26, 57/04

U.S. Cl. 260—530 N

8 Claims

## ABSTRACT OF THE DISCLOSURE

A process for producing unsaturated carboxylic acids, which comprises oxidizing unsaturated aldehydes in the vapor phase in the presence of a catalyst comprising a catalytic oxide supported on an inert carrier, such catalytic oxide containing metal elements in the atomic ratio Mo:V:Cu:Cr:W of 12:2-14:1-6:0-4:0-12 with the proviso that Cr+W is not O.

This invention relates to a process for producing unsaturated carboxylic acids. More specifically, the invention relates to a process for producing unsaturated carboxylic acids by catalytically oxidizing unsaturated aldehydes having not less than 3 carbon atoms in the vapor phase in the presence of a catalyst, for example, a process for producing acrylic acid from acrolein, or methacrylic acid from methacrolein.

Generally, in the commercial production of unsaturated carboxylic acids by the catalytic vapor phase oxidation of unsaturated aldehydes, it is of utmost importance to use catalysts which give high conversions of the unsaturated aldehydes and high selectivities to unsaturated carboxylic acids. It is required that the catalysts should be very easily produced on a commercial basis and have stability over prolonged periods of time.

Examples of the conventional catalysts for use in the production of acrylic acid or methacrylic acid by the catalytic vapor phase oxidation of acrolein or methacrolein include a catalytic oxide composed of molybdenum and vanadium as disclosed in Japanese Patent Publication No. 1,775/66, and a catalytic oxide composed of molybdenum, vanadium, aluminum and copper as disclosed in Japanese Patent Publication No. 26,287/69. The specification of Japanese Patent Publication No. 1,775/66 discloses that with the catalyst used there, the maximum one-pass yield of acrylic acid is 76.4%. Such a yield is still unsatisfactory for commercial operation. According to the specification of Japanese Patent Publication No. 26,287/69, the yield of acrylic acid can be 97-97.5% at a space velocity of 500 to 1000 hr.<sup>-1</sup> when aluminum sponge is used as a carrier and the catalyst is used in a strongly reduced condition by pre-treatment (in a state where oxygen is insufficient). However, when the space velocity is reduced to 2000 hr.<sup>-1</sup>, the yield abruptly goes down to 89.5%. In addition, the pretreatment for strongly reducing the catalysts includes a step of treating the catalyst with a reaction gas at a temperature higher than the reaction temperature, and therefore, various difficulties are encountered.

Accordingly, an object of the present invention is to provide a process for producing unsaturated carboxylic acids, which can be operated on a commercial basis using a novel catalyst.

It has now been found that by using a catalytic oxide comprising molybdenum, vanadium, copper, chromium, and/or tungsten, and oxygen supported on an inert carrier, unsaturated carboxylic acid, for example acrylic acid or methacrylic acid can be obtained in very high one-pass yields from unsaturated aldehydes, for example acrolein or methacrolein, and the above object of the present invention can be achieved.

## 2

The catalytic oxide used in the present invention is characterized in that the metallic elements which constitute it are present in the following atomic ratios:

$$\text{Mo:V:Cu:Cr:W} = 12:2-14:1-6:0-4:0-12$$

5 (with the proviso Cr+W≠O). Oxygen in the catalytic oxide need not be present in a specially reduced condition. It is assumed that oxygen is present in the catalytic oxide in the form of a complex metal oxide or metal acid salt. Therefor, the amount of oxygen present in the catalytic oxide varies according to the atomic ratios of the metal elements that constitute the catalytic oxide.

As the inert carrier for supporting the catalytic oxide in the present invention, natural, inert porous substances, may be exemplified, or inert porous substances. Specific examples include alpha-alumina, silicon carbide, pumice, silica, zirconia, titanium oxide, or mixtures of these. The inert carrier that is conveniently used in the present invention has a surface area of not more than 2 m.<sup>2</sup>/g. and a porosity of 30 to 65%, at least 90% of the pores having a pore diameter in the range of 50 to 1500 microns.

20 The catalyst used in the present invention can be prepared for example by adding an aqueous solution of ammonium bichromate and an aqueous solution of copper nitrate to an aqueous solution containing ammonium molybdate, ammonium paratungstate, and ammonium metavanadate, pouring a carrier material into the mixture, heating the mixture to evaporate it to dryness and thereby to deposit the compounds on the carrier, if desired molding it into tablets for instance, and then calcining it at 350-600° C. Any compound which can form a catalytic oxide by calcination such as hydroxides or carbonates can be used as materials for the production of the catalysts.

25 The catalytic vapor phase oxidation process of the present invention can be performed by passing a gaseous mixture consisting of 1 to 10% by volume of an unsaturated aldehyde (for example, acrolein, or methacrolein), 5 to 15% by volume of molecular oxygen, 20 to 60% by volume of steam, and 20 to 50% by volume of an inert gas over the catalyst prepared as above described, at a temperature of 200 to 350° C. and a pressure of atmospheric pressure to 10 atmospheres. The space velocity is maintained at 500 to 5000 hr.<sup>-1</sup>. The reaction can be 30 carried out either in a fixed bed or in a fluidized bed.

35 According to the present invention, the one-pass yield of the unsaturated carboxylic acid can be maintained high without a decrease in the space velocity. While not wishing to be limited by any theory, it is assumed that this is 40 perhaps because the catalytic activity is regulated by the bonding of complete oxides of copper, chromium, and tungsten or acid salts with the Mo-V system, and that it is controlled by the porosity of the carrier.

45 The invention will be described in detail by the following Examples and Comparative Examples which are presented for illustrative, rather than limitative, purposes.

The conversion, selectivity, and one-pass yield used in the present specification and claims are defined as follows:

50 Conversion (percent)

$$= \frac{\text{Moles of an unsaturated aldehyde reacted}}{\text{Moles of an unsaturated aldehyde fed}} \times 100$$

55 Selectivity (percent)

$$= \frac{\text{Moles of an unsaturated carboxylic acid produced}}{\text{Moles of an unsaturated aldehyde reacted}} \times 100$$

60 One-pass yield (percent)

$$= \frac{\text{Moles of an unsaturated carboxylic acid produced}}{\text{Moles of an unsaturated aldehyde fed}} \times 100$$

**3**  
**EXAMPLE 1**

While 5000 ml. of water were being heated with stirring, 104 g. of ammonium paratungstate, 86 g. of ammonium metavanadate, 338 g. of ammonium molybdate, and 12 g. of ammonium bichromate were added to the water. Separately, an aqueous solution of 86 g. of copper nitrate in 300 ml. of water was prepared, and mixed with the aqueous solution obtained above. The mixed solution obtained was put into a porcelain evaporator on a warm bath, and 1000 ml. of particulate alpha-alumina having a diameter of 3 to 5 mm. (surface area 1 m.<sup>2</sup>/g. or less,

**4****Comparative Example 2**

The procedure of Example 1 was repeated except that ammonium paratungstate and ammonium bichromate were not used. As a result a catalyst in which a catalytic oxide having a metal element composition of



deposited on alpha-alumina was obtained. Using this catalyst, the reaction was performed under the same conditions as set forth in Example 1. The results obtained are given in Table 1.

TABLE 1

|                       | Atomic ratio of metal elements in catalytic oxide |     |     |     |     | Reaction temperature (°C.) | Space velocity (hr. <sup>-1</sup> ) | Acrolein conversion (mol percent) | Acrylic acid selectivity (mol percent) | Acrylic acid one-pass yield (mol percent) |
|-----------------------|---------------------------------------------------|-----|-----|-----|-----|----------------------------|-------------------------------------|-----------------------------------|----------------------------------------|-------------------------------------------|
|                       | Mo                                                | V   | Cu  | Cr  | W   |                            |                                     |                                   |                                        |                                           |
| Example 1             | 12                                                | 4.6 | 2.2 | 0.6 | 2.4 | 220                        | 1,000                               | 100                               | 98.0                                   | 98.0                                      |
|                       |                                                   |     |     |     |     | 240                        | 2,000                               | 99.5                              | 98.0                                   | 97.5                                      |
|                       |                                                   |     |     |     |     | 260                        | 3,000                               | 99.0                              | 98.2                                   | 97.2                                      |
| Comparative Example 1 | 12                                                | 4.6 | 0   | 0   | 0   | 220                        | 1,000                               | 49.5                              | 40.0                                   | 19.8                                      |
|                       |                                                   |     |     |     |     | 240                        | 2,000                               | 45.0                              | 46.5                                   | 20.9                                      |
|                       |                                                   |     |     |     |     | 260                        | 3,000                               | 38.0                              | 51.0                                   | 19.4                                      |
| Comparative Example 2 | 12                                                | 4.6 | 2.2 | 0   | 0   | 220                        | 1,000                               | 54.6                              | 92.0                                   | 50.2                                      |
|                       |                                                   |     |     |     |     | 240                        | 2,000                               | 46.3                              | 93.0                                   | 43.1                                      |
|                       |                                                   |     |     |     |     | 260                        | 3,000                               | 40.0                              | 93.0                                   | 37.2                                      |

porosity 42%, and 92% of the pores being of a pore diameter 75-250 microns) were added as a carrier. With stirring, the mixture was evaporated to dryness to deposit the compounds on the carrier, and then calcined for 5 hours at 400° C. As a result a catalyst in which a catalytic oxide having a metal element composition of



deposited on the alpha-alumina carrier was obtained.

One thousand milliliters of the resulting catalyst were packed into a U-shaped stainless steel tube having a diameter of 25 cm., and the tube was immersed in a molten nitrate bath heated at 220-260° C. A gaseous mixture consisting of 4% of acrolein, 55% of air, and 41% of steam, all by volume, was fed into the tube, and reacted at a space velocity of 1000 to 3000 hr.<sup>-1</sup>. The results obtained are shown in Table 1.

**EXAMPLES 2 AND 3**

Using the same catalyst as set forth in Example 1, the reaction was performed under the same conditions as in Example 1 except that the space velocity was changed to 4000 hr.<sup>-1</sup> (Example 2) and 5000 hr.<sup>-1</sup> (Example 3). The results are given in Table 2 below.

TABLE 2

| Examples | Space velocity (hr. <sup>-1</sup> ) | Reaction temperature (°C.) | Conversion of acrolein (mole percent) | Selectivity of acrylic acid (mole percent) | One-pass yield of acrylic acid (mole percent) |
|----------|-------------------------------------|----------------------------|---------------------------------------|--------------------------------------------|-----------------------------------------------|
| 2        | 4,000                               | 270                        | 98.5                                  | 98                                         | 96.5                                          |
| 3        | 5,000                               | 270                        | 97.0                                  | 97.8                                       | 94.9                                          |

**EXAMPLES 4 TO 6**

The procedure of Example 1 was repeated except that the composition of the gaseous mixture was changed. The results obtained are given in Table 3.

TABLE 3

| Examples | Composition of gaseous mixture (vol. percent) |     |       | Reaction temperature (°C.) | Space velocity (hr. <sup>-1</sup> ) | Conversion of acrolein (mole percent) | Selectivity of acrylic acid (mole percent) | One-pass yield of acrylic acid (mole percent) |
|----------|-----------------------------------------------|-----|-------|----------------------------|-------------------------------------|---------------------------------------|--------------------------------------------|-----------------------------------------------|
|          | Acrolein                                      | Air | Steam |                            |                                     |                                       |                                            |                                               |
| 4        | 5                                             | 55  | 40    | 270                        | 4,000                               | 98.0                                  | 97.7                                       | 95.8                                          |
| 5        | 6                                             | 54  | 40    | 265                        | 3,000                               | 99.0                                  | 97.0                                       | 96.0                                          |
| 6        | 8                                             | 62  | 30    | 265                        | 3,000                               | 98.5                                  | 96.1                                       | 94.7                                          |

**Comparative Example 1**

The procedure of Example 1 was repeated except that ammonium paratungstate, ammonium bichromate, and copper nitrate were not used. As a result a catalyst in

60 Table 4 was obtained. The procedure of Example 1 was repeated except that a different carrier was used. The results are given in Table 4.

TABLE 4

| Example | Carrier                         | Physical properties of the carrier |                    |                             | Reaction temperature (°C.) | Space velocity (hr. <sup>-1</sup> ) | Conversion of acrolein (mole percent) | Selectivity of acrylic acid (mole percent) | One-pass yield of acrylic acid (mole percent) |
|---------|---------------------------------|------------------------------------|--------------------|-----------------------------|----------------------------|-------------------------------------|---------------------------------------|--------------------------------------------|-----------------------------------------------|
|         |                                 | Surface area (m. <sup>2</sup> /g.) | Porosity (percent) | Pore distribution           |                            |                                     |                                       |                                            |                                               |
| 7       | Silicon carbide                 | <1                                 | 55                 | 75-500 <sub>4</sub> , 93%   | 230                        | 2,000                               | 99.0                                  | 98.0                                       | 97.0                                          |
| 8       | α-Alumina (50%) silicon carbide | <1                                 | 47                 | 75-1,000 <sub>4</sub> , 95% | 230                        | 2,000                               | 99.0                                  | 98.0                                       | 97.0                                          |
| 9       | α-Alumina (75%) silica          | <1                                 | 40                 | 50-1,200 <sub>4</sub> , 95% | 230                        | 2,000                               | 100                                   | 98.0                                       | 98.0                                          |

which a catalytic oxide having a metal element composition  $\text{Mo}_{12}\text{V}_{4.6}$  deposited on the alpha-alumina carrier was obtained. Using this catalyst, the reaction was performed under the same conditions as set forth in Example 1. The results obtained are given in Table 1.

**EXAMPLES 7 TO 9**

The procedure of Example 1 was repeated except that a different carrier was used. The results are given in Table 4.

**EXAMPLES 10 TO 14**

The procedure of Example 1 was repeated except that the atomic ratio of metal elements in the catalytic oxide was varied. The results obtained are given in Table 5.

TABLE 5

| Example | Atomic ratio of metal elements in the catalytic oxide |     |     |     |     | Reaction temperature (° C.) | Space velocity (hr. <sup>-1</sup> ) | Conversion of acrolein (mol percent) | Selectivity of acrylic acid (mol percent) | One-pass yield of acrylic acid (mol percent) |
|---------|-------------------------------------------------------|-----|-----|-----|-----|-----------------------------|-------------------------------------|--------------------------------------|-------------------------------------------|----------------------------------------------|
|         | Mo                                                    | V   | Cu  | Cr  | W   |                             |                                     |                                      |                                           |                                              |
| 10..... | 12                                                    | 6   | 2.2 | 0   | 2.4 | 240                         | 2,000                               | 99.0                                 | 98.0                                      | 97.0                                         |
| 11..... | 12                                                    | 4.6 | 2.2 | 0.4 | 4   | 250                         | 2,000                               | 98.0                                 | 97.5                                      | 95.6                                         |
| 12..... | 12                                                    | 6   | 2.2 | 1.2 | 0   | 240                         | 2,000                               | 99.5                                 | 98.0                                      | 97.5                                         |
| 13..... | 12                                                    | 4.6 | 4.4 | 0.6 | 2.4 | 240                         | 2,000                               | 98.5                                 | 98.0                                      | 96.5                                         |
| 14..... | 12                                                    | 8   | 2.2 | 0.8 | 1.0 | 230                         | 2,000                               | 100                                  | 97.5                                      | 97.5                                         |

The results obtained in Examples 1 to 14 above demonstrate that the reaction can be performed under a wide range of conditions without reducing the yield of acrylic acid.

### EXAMPLE 15

Using the same catalyst and apparatus as used in Example 1, a gaseous mixture consisting of 4% by volume of methacrolein, 51% of air, and 45% of steam was reacted at 340° C. and a space velocity of 2000 hr.<sup>-1</sup>. The conversion of methacrolein was 70%; the selectivity of methacrylic acid was 75.5%; and the one-pass yield of methacrylic acid was 52.8%.

What is claimed is:

1. A process for producing unsaturated carboxylic acids, which comprises oxidizing unsaturated aldehydes in the vapor phase in the presence of a catalyst comprising a catalytic oxide supported on an inert carrier, said catalytic oxide consisting essentially of the recited metal elements in the atomic ratio Mo:V:Cu:Cr:W of 12:2-14:1-6:0-4:0-12 with the proviso that Cr+W is not O, said inert carrier having a surface area not greater than 2 m.<sup>2</sup>/g. and a porosity of 30 to 65%, at least 90% of the pores having a pore diameter in the range of 50 to 1500 microns.

2. A process for producing unsaturated carboxylic acids, which comprises oxidizing unsaturated aldehydes in the vapor phase at 200 to 350° C. and normal atmospheric pressure to 10 atmospheres in the presence of a catalyst comprising a catalytic oxide supported on an inert carrier, said catalytic oxide consisting essentially of the recited metal elements in the atomic ratio Mo:V:Cu:Cr:W of 12:2-14:1-6:0-4:0-12 with the proviso that Cr+W is not O, said inert carrier having a surface area not greater than 2 m.<sup>2</sup>/g. and a porosity of 30 to 65%, at least 90% of the pores having a pore diameter in the range of 50 to 1500 microns.

3. A process for producing acrylic acid, which comprises oxidizing acrolein with molecular oxygen in the vapor phase at 200-350° C. and normal atmospheric pressure to 10 atmospheres in the presence of a catalyst comprising a catalytic oxide supported on an inert carrier, said catalytic oxide consisting essentially of the recited metal elements in the atomic ratio Mo:V:Cu:Cr:W of 12:2-14:1-6:0-4:0-12 with the proviso that Cr+W is not O, said inert carrier having a surface area not greater than 2 m.<sup>2</sup>/g. and a porosity of 30 to 65%, at least 90%

of the pores having a pore diameter in the range of 50 to 1500 microns.

4. A process for producing methacrylic acid, which comprises oxidizing methacrolein with molecular oxygen in the vapor phase at 200 to 350° C. and normal atmospheric pressure to 10 atmospheres in the presence of a catalyst comprising a catalytic oxide supported on an inert carrier, said catalytic oxide consisting essentially of the recited metal elements in the atomic ratio Mo:V:Cu:Cr:W of 12:2-14:1-6:0-4:0-12 with the proviso that Cr+W is not O, said inert carrier having a surface area not greater than 2 m.<sup>2</sup>/g. and a porosity of 30 to 65%, at least 90% of the pores having a pore diameter in the range of 50 to 1500 microns.

5. The process of claim 1 wherein said inert carrier is selected from  $\alpha$ -alumina, silicon carbide, pumice, silica, zirconia, titanium oxide or mixtures thereof.

6. The process of claim 2 wherein said inert carrier is selected from  $\alpha$ -alumina, silicon carbide, pumice, silica, zirconia, titanium oxide and mixtures thereof.

7. The process of claim 3 wherein said inert carrier is selected from  $\alpha$ -alumina, silicon carbide, pumice, silica, zirconia, titanium oxide or mixtures thereof.

8. The process of claim 4 wherein said inert carrier is selected from  $\alpha$ -alumina, silicon carbide, pumice, silica, zirconia, titanium oxide or mixtures thereof.

### References Cited

#### UNITED STATES PATENTS

|           |         |                       |           |
|-----------|---------|-----------------------|-----------|
| 3,567,773 | 3/1971  | Yamaguchi et al. .... | 260-530 N |
| 3,644,509 | 2/1972  | Allen ....            | 260-530 N |
| 3,775,474 | 11/1973 | O'Hara et al. ....    | 260-530 N |

#### FOREIGN PATENTS

|           |         |                    |           |
|-----------|---------|--------------------|-----------|
| 1,924,496 | 11/1969 | Germany ....       | 260-530 N |
| 1,007,405 | 10/1965 | Great Britain .... | 260-530 N |
| 1,032,261 | 6/1966  | Great Britain .... | 260-530 N |
| 1,084,143 | 9/1967  | Great Britain .... | 260-530 N |
| 1,086,523 | 10/1967 | Great Britain .... | 260-530 N |
| 746,202   | 8/1970  | Belgium ....       | 260-530 N |

LORRAINE A. WEINBERGER, Primary Examiner

RICHARD D. KELLY, Assistant Examiner

U.S. Cl. X.R.

252—456, 464, 467

UNITED STATES PATENT OFFICE  
CERTIFICATE OF CORRECTION

Patent No. 3,833,649 Dated September 3, 1974

Inventor(s) Masahiro WADA ET AL

It is certified that error appears in the above-identified patent  
and that said Letters Patent are hereby corrected as shown below:

In the Heading, insert patentees' Foreign Application Priority  
Data as follows:

-- Claims priority, application Japan, October 23, 1970,

No. 45-92759/70. --

Signed and Sealed this  
*twenty-third Day of March 1976*

[SEAL]

Attest:

**RUTH C. MASON**  
*Attesting Officer*

**C. MARSHALL DANN**  
*Commissioner of Patents and Trademarks*

UNITED STATES PATENT OFFICE  
CERTIFICATE OF CORRECTION

Patent No. 3,833,649

Dated September 3, 1974

Inventor(s) Masahiro Wada et al.

It is certified that error appears in the above-identified patent and that said Letters Patent are hereby corrected as shown below:

The term of this patent subsequent to November 27, 1990 has been disclaimed.

Signed and Sealed this  
Eighth Day of February 1977

[SEAL]

*Attest:*

**RUTH C. MASON**  
*Attesting Officer*

**C. MARSHALL DANN**  
*Commissioner of Patents and Trademarks*